

# UNITED STATES PATENT OFFICE.

PAUL LÉON HULIN, OF GRENOBLE, FRANCE, ASSIGNOR TO SOCIÉTÉ D'ELECTRO-CHIMIE, OF PARIS, FRANCE, AND PAUL LEON HULIN, OF GRENOBLE, FRANCE.

## PROCESS FOR THE MANUFACTURE OF METALLIC SODIUM.

971,198.

Specification of Letters Patent. Patented Sept. 27, 1910.

No Drawing. Original application filed October 27, 1908, Serial No. 459,728. Divided and this application filed June 2, 1909. Serial No. 499,737.

To all whom it may concern:

Be it known that I, PAUL LÉON HULIN, of 6 Rue Félix Poulat, Grenoble, Tsère, Republic of France, engineer, have invented a 5 Process for the Manufacture of Metallic Sodium, of which the following is a full, clear, and exact description, this being a division of my application for Letters Patent for means for the electrolytic manufacture of 10 sodium, Serial No. 459,728, filed October 27, 1908.

It has been noticed in the manufacture of sodium, by means of the electrolysis of fixed caustic soda, that during the carrying out of 15 the process, the quantity of sodium produced decreases somewhat after a short time. This phenomenon cannot be attributed to an increase in the resistance of the bath, nor to the surface of the electrodes. Up till now it 20 has been surmised that the decrease in the production was due to impurities in the caustic soda, silicic acid, iron oxid, etc., which are contained even in the purest soda, the proportion of the impurities increasing 25 as the decomposition of the soda is carried out. This supposition was apparently confirmed by the fact that the quantity of sodium produced decreased all the more rapidly when the soda was very impure. Under 30 these conditions the disadvantage could only be remedied by taking the electrolytic vat out of circuit, to dismount and clean it, as soon as its efficiency began to decrease, then refilling it with new caustic soda and 35 putting it to work again. It is easy to imagine the loss of time and the considerable labor necessitated by such a process; moreover, to obviate the too frequent dismounting, and cleansing operations, only soda of the 40 purest grade was used which is very expensive, and had to be rejected when it had only supplied a small quantity of sodium. The new process does away with these disadvantages and enables sodium to be produced in 45 a practical manner and under economical conditions by electrolytic means.

The principle of the process consists in intermittently taking the cathode out of the bath, in bringing it into contact with water 50 or with any solution of aqueous nature and

then to replace it in position. Such water or solution constitutes a restorative liquid. By this process the working remains regular, the decrease in the production is arrested and the inconvenience, due to the frequent replacement of the caustic soda and to the dismounting of the whole apparatus, is entirely removed.

It should be noted that in the present case there is not visible manifestation of dirt 60 deposition on the cathode and that the new process cannot be compared to other electrolytic cases where incrustations are formed on the electrodes. It should also be remarked that, on the contrary, in certain 65 electrolytic operations and particularly in the preparation of chlorates, the formation of deposits on the cathode is considered as favorable to the efficient working of the operation.

### Claims:

1. The herein described process for the manufacture of metallic sodium, which consists in subjecting fused caustic soda to electrolysis, withdrawing the cathode periodically, bringing it into contact with a restorative liquid, and then replacing it for continuing the electrolytic operation.

2. The herein described process for the manufacture of metallic sodium, which consists in subjecting fused caustic soda to electrolysis, withdrawing the cathode periodically, bringing it into contact with water to restore its efficiency, and then replacing it for continuing the electrolytic operation.

3. The herein described process for the manufacture of metallic sodium, which consists in subjecting fused caustic soda to electrolysis, withdrawing the cathode when its efficiency becomes materially diminished, and continuing the electrolytic operation with a cathode of greater efficiency.

The foregoing specification of my process for the manufacture of metallic sodium signed by me this seventeenth day of May 95 1909.

PAUL LEON HULIN.

### Witnesses:

DEAN B. MASON,  
R. EHRIG.